

## UNITED STATES PATENT OFFICE

2,132,366

PROCESS OF BATING SKINS IN LEATHER  
MANUFACTUREJohn Arthur Wilson, Milwaukee, Wis., assignor,  
by mesne assignments, to Monsanto Chemical  
Company, a corporation of DelawareNo Drawing. Application May 10, 1935,  
Serial No. 20,770

5 Claims. (Cl. 195—6)

This invention relates to tanning processes and materials, and has for its object certain improvements in the bathing operation as applied to the treatment of hides and skins in the manufacture 5 of leather.

The action of the known digestive enzymes in the bathing process has for its object the attack and disintegration of some fraction of the hide or skin and the removal of specific structures 10 which affect the appearance of the grained surface of the finished leather.

Bathing is carried on just prior to the tanning operation, and is effected by means of a pancreatic enzyme which is most effective at a pH 15 value of 7.4. The skins contain lime when entering the bate liquor, and the diffusion of the lime into the liquor makes it alkaline. A method now in use to keep the pH value at 7.4 is to add sulfuric acid to the liquor during the entire period of bathing, regulating the flow of acid according to measurements of the pH value every 2 or 20 3 minutes.

The necessity for such frequent measurements of pH makes control difficult and introduces an 25 element of danger if the work is not done with great accuracy.

I have now found that certain alkali metal polyphosphates, also referred to herein as molecularly dehydrated alkali metal phosphates, may 30 be used in the bate bath with great advantage as to the product obtained and remarkable simplicity in the control of the bathing operation itself.

Those phosphates which I have found to be of 35 value in my process comprise the water-soluble forms of the alkali metal metaphosphates or alkali metal pyrophosphates, or mixtures of the two in varying proportion. Loose mixtures of these two classes of phosphates may be used, particularly when employing the acid pyrophosphate; but where ease in handling these products is a consideration, I may employ fused mixtures of meta and tetra pyrophosphates. These products may be made by mixing together varying 40 proportions of mono-alkali metal and di-alkali metal orthophosphates, heating the mixture to the fusion point, and quickly cooling the same. See British patent, No. 378,345, of 1932. Such treatment of the mixtures of meta and pyrophosphates 45 results in the formation of soluble polyphosphates which are new compounds, a chemical combination having occurred between the constituents of such mixtures, and it has been found that the water-soluble fused mixtures have enhanced buf-

fering properties not possessed by the loose mixtures of the constituent salts.

While generally I may employ any alkali metal dehydrated polyphosphate, I prefer to use the sodium salts because of their relative cheapness 5 and commercial availability.

The bathing liquor is made to contain from 1 to 10 grams per liter of, say, sodium polyphosphate having a pH in 1% solution of 7.10. The quantity of the phosphate employed may be varied over a considerable range, which will be dependent upon the alkali present in the hides. The bathing bath is prepared by making a solution of the phosphate described above, immersing the hides therein, and by means of acid additions adjusting the pH to 15 7.4, which is the optimum hydrogen ion concentration for the action of the digestive enzyme. The pancreatic enzyme is then added to the bath and bathing continued over a period of, say, 60 minutes. 20

I have carried out a series of comparable bathing experiments which illustrate the use of my improved process. A control test in which no phosphate was employed required the continuous addition of acid over the period of the test. 25

When 1 gram per liter of either the sodium polyphosphate described above or tetra sodium pyrophosphate was used, only occasional small additions of acid were required, the pyrophosphate requiring slightly more than the metaphosphate. 30

When 5 grams per liter of either phosphate were present in the bate bath, no further additions of acid were required.

When no phosphate was used in bathing, the calcium oxide content of the bated stock on the dry basis was 1.31%; with 1 gram per liter of sodium polyphosphate, it was 1.14%; with 5 grams, 1.13%; and with 10 grams, it was 0.59%. With 1 gram of pyrophosphate it was 1.25%; with 40 5 grams, 0.62%; and with 10 grams, it was 0.69%. 35

I have described above certain results obtained in the bathing operation using a sodium polyphosphate having a pH in 1% water solution of 7.10. Such product is commercially available at present, 45 and will contain the stoichiometric equivalent of a mixture of 80% sodium metaphosphate and 20% tetra sodium pyrophosphate. Because of the method of manufacture, which involves a fusion of the constituent salts or their equivalents followed by quickly cooling the same, the pyrophosphate has lost its chemical identity, having become merged with the metaphosphate constituent, forming the new polyphosphate. Varying proportions of the two constituents may, of 50 55

course, be employed to form the new molecularly dehydrated polyphosphates and the resultant hydrogen ion effect considerably modified. The range of hydrogen ion concentrations which may be obtained may be varied from the lower value of about 6.3 for sodium metaphosphate to an upper value of 10.6 for tetra sodium pyrophosphate. The product as produced commercially may contain small amounts of sodium orthophosphate and also acid sodium pyrophosphate present as impurities.

In many cases I may employ boric acid in conjunction with the phosphates herein mentioned. I have found that the amount of sulfuric acid required to neutralize the lime in the hides varies from 2 to 20 pounds per pack of skins. This is due to variations in the lime content. For convenience in application, I find it desirable to prepare three different grades of bates, as follows:

- 20 For stock of low lime content I prefer to employ a mixture of 88% boric acid, 10% sodium acid pyrophosphate, and 2% concentrated enzyme. Approximately 1.5 pounds of this mixture is employed per 1000 pounds of stock.
- 25 For stock of medium lime content I prefer to use a mixture of 94% boric acid, 5% sodium acid pyrophosphate, and 1% concentrated enzyme. Approximately 3 pounds of this mixture is employed per 1000 pounds of stock.
- 30 For stock of high lime content I prefer to use a mixture of 97% boric acid, 2.5% sodium acid pyrophosphate, and 1% concentrated enzyme. Approximately 6 pounds of this mixture would be employed per 1000 pounds of stock.
- 35 While I have described above certain specific

forms of my invention, it will be appreciated that it is susceptible to various changes and modifications without departing from the spirit thereof, and I desire, therefore, that it be not limited except as indicated by the prior art or as particularly pointed out in the claims. 5

What I claim is:

1. A process for bathing hides including treating said hides with a solution comprising a pancreatic digestive enzyme having hide bathing properties, 10 and a water soluble alkaline compound of sodium meta phosphate and tetra sodium pyrophosphate.
2. A process for bathing hides including treating said hides with a solution comprising a pancreatic digestive enzyme having hide bathing properties and a water soluble compound of sodium meta phosphate and tetra sodium pyrophosphate, 15 said compound having a pH value greater than 7.0.
3. A process for bathing hides including treating 20 said hides with a solution comprising a pancreatic digestive enzyme having hide bathing properties and a water soluble compound of sodium meta phosphate and sodium pyrophosphate, said solution being maintained during bathing at a pH 25 in the neighborhood of 7.4.
4. A process for bathing hides, including treating said hides with a solution comprising a pancreatic digestive enzyme and a water soluble alkali metal polyphosphate. 30
5. A process for bathing hides comprising treating said hides in water with a pancreatic digestive enzyme and a water soluble sodium polyphosphate.

JOHN ARTHUR WILSON. 35